

## UNITED STATES PATENT OFFICE

2,286,866

## MAGNESIUM BASE ALLOY

John C. McDonald, Midland, Mich., assignor to  
The Dow Chemical Company, Midland, Mich.,  
a corporation of Michigan

No Drawing. Application December 23, 1940,  
Serial No. 371,370

2 Claims. (Cl. 75—168)

The invention relates to magnesium base alloys and more particularly concerns an alloy of this nature having a high degree of formability associated with other desirable physical properties, such as excellent tensile and yield strengths.

Magnesium base alloys are being widely used in the structural arts where a light weight metal is highly desirable, such as for use in making castings, forgings, and the like. However, the use of these alloys in the rolled form to make sheet metal articles requiring forming operations, such as bending, drawing, and the like, has not progressed as rapidly due to the fact that, in general, alloys having good formability or ductility permitting relatively sharp bends to be made without the article developing external cracks, usually have inferior characteristics as regards their tensile and yield strengths.

It is, accordingly, the principal object of the invention to provide a magnesium base alloy which can be made into rolled sheet and the like

manifest over the entire range of composition indicated, I have found that, in general, when the alloy contains from about 0.1 to 0.7 per cent of cerium, 0.05 to 0.5 per cent of calcium, from 3 to 7 per cent of cadmium, and from 1.5 to 2.5 per cent of manganese, it possesses the most desirable combination of properties. A particularly desirable alloy composition contains about 0.4 per cent of cerium, 0.15 per cent of calcium, 5 per cent of cadmium, and 2 per cent of manganese, the balance being magnesium.

The following table listing some of the properties of rolled sheet metal made from my new quintary alloy and comparing these properties with those of closely related quaternary alloys illustrates the improvement in tensile and yield strengths of my new alloy over that of the related commercial alloys.

In the table the per cent elongation is to be regarded as a measure of the ductility or formability of the alloy.

Table

| Nominal composition in percent<br>(magnesium=remainder) |      |     |     | Annealed                             |                                      |                                        | Cold rolled                          |                                        |
|---------------------------------------------------------|------|-----|-----|--------------------------------------|--------------------------------------|----------------------------------------|--------------------------------------|----------------------------------------|
| Ce                                                      | Ca   | Cd  | Mn  | Percent<br>elongation<br>in 2 inches | Yield<br>strength in<br>lbs./sq. in. | Tensile<br>strength in<br>lbs./sq. in. | Yield<br>strength in<br>lbs./sq. in. | Tensile<br>strength in<br>lbs./sq. in. |
| 0.08                                                    | 0.08 | 5.0 | 2.7 | 20                                   | 27,000                               | 39,000                                 | 38,000                               | 44,000                                 |
| 0.11                                                    | 0.08 | 5.0 | —   | 21                                   | 22,000                               | 36,000                                 | 31,000                               | 39,000                                 |
| 0.11                                                    | 0.11 | —   | 2.2 | 19                                   | 25,000                               | 33,000                                 | 34,000                               | 41,000                                 |

possessing a high degree of ductility or formability at ordinary temperatures permitting it to be sharply bent, drawn, or otherwise shaped, while also having highly improved tensile and yield strengths.

Other objects and advantages will be apparent as the description of the invention proceeds.

My invention resides in the discovery that a magnesium base alloy containing from about 0.01 to 1 per cent of cerium, 0.01 to 1 per cent of calcium, 1 to 12 per cent of cadmium, and from about 0.01 to 3 per cent of manganese possesses the aforementioned improved properties. The term "magnesium" used herein and in the appended claims is intended to include magnesium containing the ordinary impurities that are found in the commercially pure metal, such as traces of iron, copper, nickel, and silicon. While the properties of highly improved tensile and yield strengths coupled with excellent formability are

40 The properties set forth above under the term "annealed" were obtained by first rolling specimens at a temperature of 600° F. and thereafter annealing them at various temperatures in a range of from 400 to 800° F. The properties selected for the table were those of the annealed specimens which exhibited the maximum elongation. The properties set forth under the term "cold rolled" were obtained by subjecting specimens of the alloys, which had first been hot rolled at a temperature of 600° F., to additional rolling in the cold state. The properties selected for the table were those of the cold rolled specimens which exhibited the greatest tensile and yield strengths, while having at least a 1 per cent elongation in 2 inches.

45 A comparison of the properties listed in the table shows that the tensile and yield strengths of my new alloy are superior to those of closely related alloys, while the ductility or formability

as represented by the per cent elongation is also of a high order. A corresponding improvement is exhibited throughout the composition range of the alloying ingredients indicated.

While the new alloy is most useful in wrought form, due to its formability characteristics it may also be suitably used in making castings, extruded forms, and the like.

The new alloy may be compounded by any of the methods usually employed for melting and alloying metals with magnesium, such as by adding the alloying ingredients singly or jointly to a bath of molten magnesium which is preferably protected from oxidation by a suitable flux. The flux should be substantially free from magnesium chloride if the calcium content of the alloy is above 0.3 per cent. In those instances where an alloy is to be compounded containing less than 0.3 per cent of calcium, magnesium chloride may be present in the flux, but in this case it is preferable to add the calcium last and without too much stirring and agitation in order to prevent loss of calcium into the flux. Cerium may be

added to the alloy as such, or in the form of Misch-metal. Magnesium-cerium alloys are commonly made up by employing Misch-metal as a source of cerium. It is sometimes desirable to add more than the theoretical amount of Misch-metal since the alloying efficiency is not always 100 per cent and some loss may be incurred.

It is to be understood that the invention is not limited to the specific composition herein described, but may take other forms without departing from the scope of the invention.

I claim:

1. A magnesium base alloy containing from about 0.1 to 0.7 per cent of cerium, from 0.05 to 0.5 per cent of calcium, from 3 to 7 per cent of cadmium, and from about 1.5 to 2.5 per cent of manganese, the balance being magnesium.

2. A magnesium base alloy containing 0.4 per cent of cerium, 0.15 per cent of calcium, 5 per cent of cadmium, and 2 per cent of manganese, the balance being magnesium.

JOHN C. McDONALD.